



US008652715B2

(12) **United States Patent**  
**Wu et al.**

(10) **Patent No.:** **US 8,652,715 B2**  
(45) **Date of Patent:** **Feb. 18, 2014**

(54) **LOW TORQUE OVERCOAT FOR IMAGING DEVICE**

(75) Inventors: **Jin Wu**, Pittsford, NY (US); **Lanhui Zhang**, Webster, NY (US); **Lin Ma**, Pittsford, NY (US); **Marc J. Livecchi**, Rochester, NY (US)

(73) Assignee: **Xerox Corporation**, Norwalk, CT (US)

(\*) Notice: Subject to any disclaimer, the term of this patent is extended or adjusted under 35 U.S.C. 154(b) by 400 days.

(21) Appl. No.: **12/958,432**

(22) Filed: **Dec. 2, 2010**

(65) **Prior Publication Data**

US 2012/0141930 A1 Jun. 7, 2012

(51) **Int. Cl.**  
**G03G 15/04** (2006.01)

(52) **U.S. Cl.**  
USPC ..... **430/66**; 430/56; 430/58.05

(58) **Field of Classification Search**  
USPC ..... 430/56, 58.05, 66  
See application file for complete search history.

(56) **References Cited**

U.S. PATENT DOCUMENTS

2008/0014518 A1\* 1/2008 Yanus et al. ..... 430/58.05  
2008/0107979 A1\* 5/2008 Yanus et al. ..... 430/58.2  
2009/0246657 A1\* 10/2009 Wu et al. ..... 430/58.5  
2010/0068636 A1\* 3/2010 Aziz et al. ..... 430/58.8

\* cited by examiner

*Primary Examiner* — Stewart Fraser

(74) *Attorney, Agent, or Firm* — MDIP LLC

(57) **ABSTRACT**

An overcoat containing a copolymer of a first propylene monomer and a second hydrophilic monomer provides superior wear resistance and low torque to a photoreceptor.

**10 Claims, No Drawings**

## 1

## LOW TORQUE OVERCOAT FOR IMAGING DEVICE

## FIELD

A novel overcoat for an electrostatographic imaging device component is provided. The imaging device component can be used in electrophotographic or electrostatographic devices, such as, xerographic devices.

## BACKGROUND

In the electrostatographic imaging arts, the photoactive portions of most photoreceptors now are composed of organic materials. The rigor and repetitive use thereof command durability of the components, such as, the photoreceptors.

High speed electrophotographic copiers, duplicators and printers often experience degradation of image quality over extended cycling. The high speed imaging, duplicating and printing devices place stringent requirements on the imaging device components. For example, the functional layers of modern photoreceptors must be flexible, durable, adhere well to adjacent layers and exhibit predictable electrical characteristics within narrow operating limits to provide acceptable toner images over many thousands of cycles.

A premium is placed on photoreceptor life where a major factor limiting longevity is repetitive use and wear. For example, many imaging devices now use a smaller diameter photoreceptor. The smaller diameter photoreceptors exacerbate the wear problem because, for example, several revolutions of the drum are required to image a single page.

Hence, a problem to be solved is developing photoreceptors which are durable without sacrificing the properties and functions thereof. That problem was solved by developing a copolymer-doped overcoat with lower levels of surface friction, thereby reducing torque, increasing wear resistance and extending photoreceptor life.

## SUMMARY

According to aspects disclosed herein, there is provided a photoreceptor overcoat composition comprising a film-forming material, such as, a resin, and an overcoat comprising a block copolymer comprising a first propylene monomer and a second hydrophilic monomer, such as, an alcohol.

One disclosed feature of the embodiments is a photoreceptor comprising an overcoat comprising a film-forming material, such as, a resin, and an overcoat comprising a block copolymer comprising a first propylene monomer and a second hydrophilic monomer, such as, an alcohol.

Another disclosed embodiment is an imaging or printing device comprising a photoreceptor comprising an overcoat comprising a film-forming material, such as, a resin, and an overcoat comprising a block copolymer comprising a first propylene monomer and a second hydrophilic monomer, such as, an alcohol.

## DETAILED DESCRIPTION

As used herein, the term, "electrostatographic," or grammatical versions thereof, is used interchangeably with the terms, "electrophotographic" and "xerographic." The terms, "charge blocking layer" and "blocking layer," are used interchangeably with the terms, "undercoat layer" or "undercoat," or grammatical versions thereof. "Photoreceptor," is used interchangeably with, "photoconductor," "imaging member" or "imaging component," or grammatical versions thereof.

## 2

For the purposes of the instant application, "about," is meant to indicate a deviation of no more than 20% of a stated value or a mean value.

In electrostatographic reproducing or imaging devices, 5 including, for example, a digital copier, an image-on-image copier, a contact electrostatic printing device, a bookmarking device, a facsimile device, a printer, a multifunction device, a scanning device and any other such device, a printed output is provided, whether black and white or color, or a light image of 10 an original is recorded in the form of an electrostatic latent image on an imaging device component, such as, a photoreceptor, which may be present as an integral component of an imaging device or as a replaceable component or module of an imaging device, and that latent image is rendered visible 15 using electrostatic, finely divided, colored or pigmented particles, or toner. The imaging device component or photoreceptor can be used in electrophotographic (xerographic) imaging processes and devices, for example, as a flexible belt or in a rigid drum configuration. Other components may 20 include a flexible intermediate image transfer belt, which can be seamless or seamed.

The imaging device component, the photoreceptor, generally comprises one or more functional layers. Certain photoreceptors include a photoconductive layer or layers formed on 25 an electrically conductive substrate or surface. The photoconductive layer is an insulator in the dark so that electric charge is retained on the surface thereof, which charge is dissipated on exposure to light. In some embodiments of interest, a photoreceptor includes an overcoat containing a hydrophilic 30 propylene copolymer.

One type of composite photoconductive layer used in xerography is illustrated in U.S. Pat. No. 4,265,990 which describes an imaging device component having at least two electrically operative layers, a photoconductive layer which 35 photogenerates holes and injects the photogenerated holes into a charge transport layer. The photoreceptors can carry a uniform negative or positive electrostatic charge to generate an image which is visualized with finely divided electrostatic colored or pigmented particles.

40 Embodiments of the present imaging device component or photoreceptor can be used in an electrophotographic image forming device or printing device. Hence, the imaging device component or photoreceptor is electrostatically charged and then is exposed to a pattern of activating electromagnetic 45 radiation, such as light, which dissipates the charge in the illuminated areas of the imaging device component while leaving behind an electrostatic latent image in the non-illuminated areas. The electrostatic latent image then is developed at one or more developing stations to form a visible 50 image by depositing finely divided electrostatic colored, dyed or pigmented particles, or toner, for example, from a developer composition, on the surface of the imaging component. The resulting visible image on the photoreceptor is transferred to a suitable receiving member, such as a paper.

55 Alternatively, the developed image can be transferred to an intermediate transfer device, such as a belt or a drum, and the image then is transferred to a receiving member, such as a paper, or various other receiving members or substrates, such as, a cloth, a polymer, a plastic, a metal and so on, which can be presented in any of a variety of forms, such as a flat surface, a sheet or a curved surface. The transferred colored particles are fixed or fused to the receiving member by any of a variety of means, such as, by exposure to elevated temperature and/or pressure.

60 Thus, a photoreceptor can include a support or substrate; which may comprise a conductive surface or a conductive layer or layers (which may be referred to herein as a ground

plane layer) on an inert support; a charge generating layer (CGL); a charge transport layer (CTL); and an overcoat. Other optional functional layers that can be included in a photoreceptor include a hole blocking layer; an undercoat; an adhesive interface layer; a ground strip; and an anti-curl back coating layer. It will be appreciated that one or more of the layers may be combined into a single layer.

#### The Substrate

The imaging device component substrate (or support) may be opaque or substantially transparent, and may comprise any suitable organic or inorganic material having the requisite mechanical properties. The entire substrate can comprise an electrically conductive material, or an electrically conductive material can be a coating on an inert substrate. Any suitable electrically conductive material can be employed, such as, copper, brass, nickel, zinc, chromium, stainless steel, conductive plastics and rubbers, aluminum, semitransparent aluminum, steel, cadmium, silver, gold, indium, tin, zirconium, niobium, tantalum, vanadium, hafnium, titanium, tungsten, molybdenum and so on; or a paper, a plastic, a resin, a polymer and the like rendered conductive by the inclusion of a suitable conductive material therein or thereon; metal oxides, including tin oxide and indium tin oxide; and the like. The conductive material can comprise a single of the above-mentioned materials, such as, a single metallic compound, or a plurality of materials and/or a plurality of layers of different components, such as, a metal or an oxide, plural metals; and so on.

The substrate can be an insulating material including inorganic or organic polymeric materials, such as a commercially available biaxially oriented polyethylene terephthalate, a commercially available polyethylene naphthalate and so on, with a ground plane layer comprising a conductive coating comprising one or more of the materials provided hereinabove, including a titanium or a titanium/zirconium coating, or a layer of an organic or inorganic material having a semi-conductive surface layer, such as, indium tin oxide, aluminum, titanium and the like. Thus, a substrate can be a plastic, a resin, a polymer and so on, such as, a polycarbonate, a polyamide, a polyester, a polypropylene, a polyurethane, a polyethylene and so on.

The substrate may have a number of many different configurations, such as, for example, a plate, a sheet, a film, a cylinder, a drum, a scroll, a flexible belt, which may be seamed or seamless, and the like.

The thickness of the substrate can depend on any of a number of factors, including flexibility, mechanical performance and economic considerations. The thickness of the substrate may range from about 25  $\mu\text{m}$  to about 3 mm. In embodiments of a flexible imaging belt, the thickness of a substrate can be from about 50  $\mu\text{m}$  to about 200  $\mu\text{m}$  for flexibility and to minimize induced imaging device component surface bending stress when a imaging device component belt is cycled around small diameter rollers in a machine belt support module, for example, 19 mm diameter rollers.

Generally, a substrate is not soluble in any of the solvents used in the coating layer solutions, can be optically transparent or semi-transparent, and can be thermally stable up to a temperature of about 150° C. or more.

#### The Conductive Layer

When a conductive ground plane layer is present, the layer may vary in thickness depending on the optical transparency and flexibility desired of the electrophotographic imaging device component. When an imaging flexible belt is used, the thickness of the conductive layer on the substrate, for example, a titanium and/or a zirconium conductive layer produced by sputtering, typically ranges from about 2 nm to

about 75 nm in thickness to allow adequate light transmission for proper back erase. In other embodiments, a conductive layer can be from about 10 nm to about 20 nm in thickness for a combination of, for example, electrical conductivity, flexibility and light transmission. For rear erase exposure, a conductive layer light transparency of at least about 15% can be used. The conductive layer may be an electrically conductive metal layer which may be formed, for example, on the substrate by any suitable coating technique, such as, a vacuum 10 depositing, dipping or sputtering and so on as taught herein or as known in the art, and the coating dried on the substrate using methods taught herein or known in the art. (That and any of the methods for making a layer as taught herein may be practiced for making any other layer of a photoreceptor.) 15 Typical metals suitable for use in a conductive layer include aluminum, zirconium, niobium, tantalum, vanadium, hafnium, titanium, nickel, stainless steel, chromium, tungsten, molybdenum, combinations thereof and the like. The conductive layer need not be limited to metals. Hence, other 20 examples of conductive layers may be combinations of materials such as conductive indium tin oxide as a transparent layer for light having a wavelength of between about 4000  $\text{\AA}$  and about 9000  $\text{\AA}$  or a conductive carbon black dispersed in a plastic binder as an opaque conductive layer.

#### The Hole Blocking Layer

An optional hole blocking layer may be applied, for example, to the undercoat. Any suitable positive charge (hole) blocking layer capable of forming an effective barrier to the injection of holes from the adjacent conductive layer or substrate to the photoconductive layer(s) or CGL may be used. The hole blocking layer may include polymers, such as, a polyvinylbutyral, epoxy resins, polyesters, polysiloxanes, polyamides, polyurethanes, methacrylates, such as, hydroxyethyl methacrylate (HEMA), hydroxylpropyl celluloses, 35 polyphosphazines and the like, or may comprise nitrogen-containing siloxanes or silanes, or nitrogen-containing titanium or zirconium compounds, such as, titanate and zirconate. Such film-forming materials can be used to make any of the layers taught herein. The hole blocking layer may have a 40 thickness of from about 0.2  $\mu\text{m}$  to about 10  $\mu\text{m}$ , depending on the type of material chosen as a design choice. Typical hole blocking layer materials include, for example, trimethoxysilyl propylene diamine, hydrolyzed trimethoxysilyl propyl ethylene diamine, N- $\beta$ -(aminoethyl)- $\gamma$ -aminopropyl 45 tri-methoxy silane, isopropyl 4-aminobenzene sulfonyl di(dodecylbenzene sulfonyl) titanate, isopropyl di(4-aminobenzoyl) isostearoyl titanate, isopropyl tri(N-ethylaminoethylamino) titanate, isopropyl trianthranil titanate, isopropyl tri(N,N-dimethylethylamino)titanate, titanium-4-amino benzene 50 sulfonate oxyacetate, titanium 4-aminobenzoate isostearate oxyacetate, ( $\gamma$ -aminobutyyl)methyl diethoxysilane, ( $\gamma$ -aminopropyl)methyl diethoxysilane and combinations thereof, as disclosed, for example, in U.S. Pat. Nos. 4,338,387; 4,286, 033; 4,988,597; 5,244,762; and 4,291,110, each incorporated 55 herein by reference in entirety.

The blocking layer may be applied by any suitable conventional technique, such as, spraying, dip coating, draw bar coating, gravure coating, silk screening, air knife coating, reverse roll coating, vacuum deposition, chemical treatment 60 and the like. For convenience in obtaining thin layers, the blocking layer may be applied in the form of a dilute solution, with the solvent being removed after deposition of the coating by conventional techniques, such as, vacuum, heating and the like. A weight ratio of blocking layer material and solvent of between about 0.05:100 to about 5:100 can be used for spray coating. Such deposition methods for forming layers can be used for making any of the herein described layers.

## The Adhesive Interface Layer

An optional adhesive interface layer may be employed. An interface layer may be situated, for example, intermediate between the hole blocking layer and the CGL. The interface layer may include a film-forming material, such as, a polyurethane, a polyester and so on. An example of a polyester includes a polyarylate, a polyvinylbutyral and the like.

Any suitable solvent or solvent mixture may be employed to form an adhesive interface layer coating solution. Typical solvents include tetrahydrofuran, toluene, monochlorobenzene, methylene chloride, cyclohexanone and the like, as well as mixtures thereof. Any suitable and conventional technique may be used to mix and thereafter to apply the adhesive interface layer coating mixture to the photoreceptor under construction as taught herein or as known in the art. Typical application techniques include spraying, dip coating, roll coating, wire wound rod coating and the like. Drying of the deposited wet coating may be accomplished by any suitable conventional process, such as oven drying, infrared drying, air drying and the like.

The adhesive interface layer may have a thickness of from about 0.01  $\mu\text{m}$  to about 900  $\mu\text{m}$  after drying. In certain embodiments, the dried thickness is from about 0.03  $\mu\text{m}$  to about 1  $\mu\text{m}$ .

## The Charge Generating Layer

The CGL can comprise any suitable charge generating binder or film-forming material including a charge generating/photoconductive material suspended or dissolved therein, which may be in the form of particles and dispersed in a film-forming material or binder, such as, an electrically inactive resin. Examples of charge generating materials include, for example, inorganic photoconductive materials, such as, azo materials, such as, certain dyes, such as, Sudan Red and Diane Blue, quinone pigments, cyanine pigments and so on, amorphous selenium, trigonal selenium and selenium alloys, such as, selenium-tellurium, selenium-tellurium-arsenic, selenium arsenide and mixtures thereof, germanium and organic photoconductive materials, including various phthalocyanine pigments, such as, the X form of metal-free phthalocyanine, metal phthalocyanines, such as, vanadyl phthalocyanine and copper phthalocyanine, hydroxygallium phthalocyanines, chlorogallium phthalocyanines, titanyl phthalocyanines, quinacridones, dibromo anthanthrone pigments, benzimidazole perylene, substituted 2,4-diaminotriazines, polynuclear aromatic quinones and the like, dispersed or suspended in a film-forming material, such as, a polymer, or a binder. Selenium, selenium alloy and the like and mixtures thereof may be formed as a homogeneous CGL. Benzimidazole perylene compositions are described, for example, in U.S. Pat. No. 4,587,189, the entire disclosure thereof being incorporated herein by reference. Multicharge generating layer compositions may be used where a photoconductive layer enhances or reduces the properties of the CGL. The charge generating materials can be sensitive to activating radiation having a wavelength of from about 400 nm to about 900 nm during the imagewise radiation exposure step forming an electrostatic latent image. For example, hydroxygallium phthalocyanine absorbs light of a wavelength of from about 370 nm to about 950 nm, as disclosed, for example, in U.S. Pat. No. 5,756,245.

Any suitable film-forming material may be employed in a CGL, including those described, for example, in U.S. Pat. No. 3,121,006, the entire disclosure thereof being incorporated herein by reference in entirety, or as taught herein. Typical film-forming materials include thermoplastic and thermosetting resins, such as, a polycarbonate, a polyester, a polyamide, a polyurethane, a polystyrene, a polyarylether, a polyarylsul-

fone, a polybutadiene, a polysulfone, a polyethersulfone, a polyethylene, a polypropylene, a polyimide, a polymethylpentene, a polyphenylenesulfide, a polyvinylbutyral, a polyvinyl acetate, a polysiloxane, a polyacrylate, a polyvinylacetal, an amino resin, a phenyleneoxide resin, a terephthalic acid resin, an epoxy resin, a phenolic resin, an acrylonitrile copolymer, a polyvinylchloride, a vinylchloride, a vinyl acetate copolymer, an acrylate copolymer, an alkyd resin, a cellulosic film former, a poly(amideimide), a styrene-butadiene copolymer, a vinylidenechloride/vinylchloride copolymer, a vinylacetate/vinylidene chloride copolymer, a styrene-alkyd resin and the like. Another film-forming material is PCZ-400 (poly(4,4'-dihydroxy-diphenyl-1-1-cyclohexane) with a viscosity/molecular weight of about 40,000. A copolymer can be a block or a graft, random or alternating, and so on. The materials, polymers and copolymers mentioned herein can be used in any of the layers taught herein.

The charge generating material can be present in the film-forming material or binder composition in varying amounts. Generally, from about 5% by weight or volume to about 90% by weight or volume of the charge generating material is dispersed in about 10% by weight or volume to about 95% by weight or volume of the film-forming material or binder, or from about 20% by volume to about 60% by volume of the charge generating material is dispersed in about 40% by volume to about 80% by volume of the film-forming material or binder composition.

The CGL containing the charge generating material and the binder or film-forming material generally ranges in thickness from about 0.1  $\mu\text{m}$  to about 5  $\mu\text{m}$ , for example, or from about 0.3  $\mu\text{m}$  to about 3  $\mu\text{m}$  when dry. The CGL thickness can be related to film or binder content, higher film or binder content compositions generally employ thicker layers for charge generation.

In some embodiments, the CGL may comprise a charge transport molecule or component, as discussed below in regard to the CTL. The charge transport molecule may be present in some embodiments from about 1% to about 60% by weight of the total weight of the CGL.

## The Charge Transport Layer

The CTL generally is superior or exterior to the CGL and may include any suitable film-forming material, such as, a transparent organic polymer or non-polymeric material capable of supporting the injection of photogenerated holes or electrons from the CGL and capable of allowing the transport of the holes/electrons through the CTL to selectively discharge the charge on the surface of the imaging device component, such as, a photoreceptor. The CTL can be a substantially non-photoconductive material, but one which supports the injection of photogenerated holes from the CGL. The CTL is normally transparent in a wavelength region in which the electrophotographic imaging device component is to be used when exposure is effected therethrough to ensure that most of the incident radiation is utilized by the underlying CGL. Thus, the CTL exhibits optical transparency with negligible light absorption and negligible charge generation when exposed to a wavelength of light useful in xerography, e.g., from about 400 nm to about 900 nm. In the case when the imaging device component is prepared with transparent materials, imagewise exposure or erase may be accomplished through the substrate with all light passing through the back side of the substrate. In that case, the materials of the CTL need not transmit light in the wavelength region of use if the CGL is sandwiched between the substrate and the CTL.

In one embodiment, the CTL not only serves to transport holes, but also to protect the CGL from abrasion or chemical attack and may therefore extend the service life of the imaging device component.

The CTL may include any suitable charge transport molecule or activating compound useful as an additive molecularly dispersed in an electrically inactive polymeric film-forming material or binder to form a solution and thereby making the overall material electrically active. The charge transport molecule may be added to a film-forming polymeric material, a film-forming material or binder which is otherwise incapable of supporting the injection of photogenerated holes from the charge generating material and incapable of allowing the transport of the holes therethrough. The charge transport molecule typically comprises small molecules of an organic compound which cooperate to transport charge between molecules and ultimately to the surface of the CTL, for example, see U.S. Pat. Nos. 7,759,032 and 7,704,658.

For example, N,N'-diphenyl-N,N'-bis(3-methylphenyl)-(1,1'-biphenyl)-4,4'-diamine can be used as a charge transport molecule. Other charge transport molecules include pyrazolines, diamines, hydrazones, oxadiazoles, stilbenes, carbazoles, oxazoles, triazoles, imidazoles, imidazolones, imidazolidines, bisimidazolidines, styryls, oxazolones, benzimidazoles, quinalolines, benzofurans, acridines, phenazines, aminostilbenes, aromatic polyamines, such as aryl diamines and aryl triamines, such as, aromatic diamines, including, N,N'-diphenyl-N,N'-bis(alkylphenyl)-1,1'-biphenyl-4,4'-diamines; N,N'-diphenyl-N,N'-bis[3-methylphenyl]-[1,1'-biphenyl]-4,4'-diamines; N,N'-diphenyl-N,N'-bis(chlorophenyl)-1,1'-biphenyl-4,4'-diamines; N,N'-bis-(4-methylphenyl)-N,N'-bis(4-ethylphenyl)-1,1'-3,3'-dimethylbiphenyl)-4,4'-diamines, N,N'-bis-(3,4-dimethylphenyl)-4,4'-biphenyl amines; and combinations thereof. Other suitable charge transport molecules include pyrazolines, such as, 1-[lepidyl-(2)]-3-(p-diethylaminophenyl)-5-(p-diethylaminophenyl)pyrazoline, as described, for example, in U.S. Pat. Nos. 4,315,982, 4,278,746, 3,837,851, and 6,214,514; substituted fluorene charge transport molecules, such as, 9-(4'-dimethylaminobenzylidene)fluorene, as described in U.S. Pat. Nos. 4,245,021 and 6,214,514; oxadiazole transport molecules, such as 2,5-bis(4-diethylaminophenyl)-1,3,4-oxadiazole, pyrazolines, imidazoles and triazoles, as described, for example, in U.S. Pat. No. 3,895,944; hydrazones, such as p-diethylaminobenzaldehyde (diphenylhydrazone), as described, for example, in U.S. Pat. Nos. 4,150,987, 4,256,821, 4,297,426, 4,338,388, 4,385,106, 4,387,147, 4,399,207, 4,399,208 and 6,124,514; and tri-substituted methanes, such as, alkyl-bis(N,N-dialkylaminoaryl) methanes, as described, for example, in U.S. Pat. No. 3,820,989. The disclosure of each of those patents is incorporated herein by reference in entirety.

The charge transport molecule may be present in some embodiments from about 1% to about 70% by weight of the total weight of the CTL or in other embodiments from about 10% to about 70% by weight of the total weight of the CTL, or from about 20% to about 70%; from about 30% to about 70%; or from about 40% to about 70% of the total weight of the CTL.

Any suitable electrically inactive film-forming material or binder may be used to form the CTL. Typical inactive film-forming materials or binders include, a polycarbonate resin, a polystyrene, a polyester, a polyarylate, a polyacrylate, a polyether, a polyethylene, which may be substituted, for example, with a hydrocarbon or a halogen, a polysulfone, a fluorocarbon, a thermoplastic polymer and the like. Molecular weights can vary, for example, from about 20,000 to about 150,000.

Examples of film-forming materials or binders include a polycarbonate, such as, poly(4,4'-isopropylidene-diphenylene)carbonate (referred to as bisphenol-A-polycarbonate or PCA), poly(4,4'-cyclohexylidene-diphenylene) carbonate (referred to as bisphenol-Z-polycarbonate or PCZ), poly(4,4'-isopropylidene-3,3'-dimethyl-diphenyl)carbonate (referred to as bisphenol-C-polycarbonate or PCC) and the like and mixtures thereof.

Lubricating agents can be included in a CTL. Suitable lubricants include a polyether (for example, see U.S. Pat. No. 7,427,440); one with antioxidant activity, as taught, for example, in U.S. Pat. No. 7,544,451; a phosphorus-containing compound, such as phosphite or a phosphoric acid amine salt, for example, as provided in U.S. Pat. No. 7,651,827; a synthetic hydrocarbon; a polyolefin; a polyester; a thiocarbonate; a fluorinated resin, such as, a polytetrafluoroethylene (PTFE); copolymers of a fluorinated resin, such as, a copolymer of tetrafluoroethylene and hexafluoropropylene, a copolymer of tetrafluoroethylene and perfluoro(propyl vinyl ether), a copolymer of tetrafluoroethylene and perfluoro(ethyl vinyl ether), a copolymer of tetrafluoroethylene and perfluoro(methyl vinyl ether), a copolymer of tetrafluoroethylene, hexafluoropropylene and vinylidene fluoride, mixtures thereof, and the like, inclusive of a number of suitable known fluorinated polymers; a lamellar solid; a polyethylene; a polypropylene and so on, for example, as provided, for example, in U.S. Pat. Nos. 7,527,902 and 7,468,208.

Crosslinking agents can be used to promote polymerization of the polymer or film-forming material of a CTL. Examples of suitable crosslinking agents include an acrylated polystyrene, a methacrylated polystyrene, an ethylene glycol dimethacrylate, a bisphenol A glycerolate dimethacrylate, a (dimethylvinylsilyloxy)heptacyclopentyltricycloheptasiloxanediol and the like and mixtures thereof. The crosslinking agent can be used in an amount of from about 1% to about 20%, from about 5% to about 10%, or from about 6% to about 9% by weight or volume of total polymer or film-forming material content.

The CTL can contain variable amounts of an antioxidant, such as a hindered phenol. An example of a hindered phenol is octadecyl-3,5-di-tert-butyl-4-hydroxyhydrocinnamate. The hindered phenol may be present in an amount of up to about 10 weight % based on the concentration or amount of the charge transport molecule. Other suitable antioxidants are described, for example, in U.S. Pat. No. 7,018,756, incorporated herein by reference in entirety.

In some embodiments, the carbonate monomer is one which is composed of one or more aryl groups. An example of such an aryl group is a bisphenol. Hence, a bisphenol compound can be polymerized into a polycarbonate by reacting same with base, such as, sodium hydroxide, and phosgene, as known in the art.

Examples of bisphenol monomers that can be used in a copolymer of interest include bisphenol A, bisphenol B, bisphenol C, bisphenol F, bisphenol S, bisphenol Z and so on.

A copolymer of interest can have a  $T_g$  of 180° C. or more; of 190° C. or more; of 200° C. or more; of 220° C. or more and so on.

The average molecular weight of a copolymer of interest can be about 10 k MW, about 40 k MW, about 70 k MW, about 100 k MW, about 120 k MW or more.

A CTL of interest can comprise a film-forming material; a charge transport material; and a lubricant. The lubricant, can be a fluorinated resin, such as a polytetrafluoroethylene (PTFE) or a copolymer of a fluorinated resin, such as, tetrafluoroethylene and hexafluoropropylene; a copolymer of tetrafluoroethylene and perfluoro(propyl vinyl ether); a

copolymer of tetrafluoroethylene and perfluoro(ethyl vinyl ether); a copolymer of tetrafluoroethylene and perfluoro(methyl vinyl ether); a copolymer of tetrafluoroethylene, hexafluoropropylene and vinylidene fluoride, mixtures thereof, and the like, inclusive of a number of suitable known fluorinated polymers, can be present in an amount, relative to the total, from about 1% to about 15%; from about 3% to about 10%; or about 8% or about 9% in a CTL of interest. The charge transport material can be present from about 20% to about 50% of the CTL; from about 25% to about 45%; from about 30% to about 40%; or about 35% in a CTL of interest. The remainder comprises a film-forming material. (The above amounts and percentages, including those presented elsewhere in the specification, are in terms of and relative to w/v, w/w or v/w as appropriate for the material(s).)

Any suitable and conventional technique may be used to mix and thereafter to apply the CTL coating mixture to the photoreceptor under construction. Typical application techniques include spraying, dip coating, roll coating, wire wound rod coating and the like. Drying of the deposited coating may be obtained by any suitable conventional technique, such as, oven drying, infrared drying, air drying and the like.

The CTL can be an insulator to the extent that the electrostatic charge placed on the CTL is not conducted in the absence of illumination at a rate sufficient to prevent formation and retention of an electrostatic latent image thereon. In general, the ratio of the thickness of the CTL to the CGL is from about 2:1 to about 200:1 and in some instances as great as about 400:1.

The thickness of the CTL can be from about 5  $\mu\text{m}$  to about 200  $\mu\text{m}$ , or from about 15  $\mu\text{m}$  to about 40  $\mu\text{m}$ . The CTL may comprise dual layers or plural layers, and each layer may contain different concentrations of a charge transporting component or may contain different charge transporting components.

#### The Ground Strip Layer

Another possible layer is a ground strip layer, including, for example, conductive particles dispersed in a film-forming material or binder, which may be applied to one edge of the imaging device component to promote electrical continuity, for example, with the conductive layer or the substrate. The ground strip layer may include any suitable film-forming material, polymer or binder and electrically conductive particles as taught herein. Typical ground strip materials include those enumerated in U.S. Pat. No. 4,664,995, the entire disclosure of which is incorporated by reference herein.

#### The Overcoat Layer

An overcoat layer of interest provides imaging device component surface protection, improved cleanability, reduced friction as well as improved resistance to abrasion, see, for example U.S. Pat. Nos. 7,833,683 and 7,759,032.

An overcoat layer can include at least a film-forming material or binder, such as, a resin, a copolymer comprising a first propylene monomer and a second hydrophilic monomer, and optionally, can include a hole transporting molecule, such as, a biphenyl or terphenyl diamine hole transporting molecule. The overcoating layer can be formed, for example, from a solution or other suitable mixture of the film-forming material or binder, such as, a resin.

The film-forming material or binder, such as, a resin, used in forming the overcoating layer can be any suitable film-forming material or binder, such as, a resin, including any of those described herein. The film-forming material or binder, such as, a resin, can be electrically insulating, semi-conductive or conductive, and can be hole transporting or not hole transporting. Thus, for example, suitable film-forming materials or binders, such as, resins, can be selected from, but are

not limited to, thermoplastic and thermosetting resins, such as, polycarbonates, polyesters, polyamides, for example, cyclic polyamides, such as, melamines, polyurethanes, polystyrenes, polyarylethers, polyamines, such as, melamines, polyarylsulfones, polysulfones, polyethersulfones, polyphenylene sulfides, polyvinyl acetates, polyacrylates, polyvinyl acetals, polyamides, polyimides, amino resins, phenylene oxide resins, phenoxy resins, epoxy resins, phenolic resins, polystyrenes, acrylonitriles, copolymers, vinyl acetate copolymers, acrylate copolymers, alkyd resins, styrenebutadiene copolymers, styrene-alkyd resins, polyvinylcarbazoles and the like. A copolymer may be block, graft, random or alternating.

In some embodiments, the film-forming material or binder, such as, a resin, can be a polyester polyol, such as, a branched polyester polyol. The prepolymer can be synthesized using a significant amount of a polyfunctional monomer, such as, trifunctional alcohols, such as triols, to form a polymer having a significant number of branches off the main polymer chain. That is distinguished from a linear prepolymer that contains only difunctional monomers, and thus little or no branches off the main polymer chain. As used herein, "polyester polyol" is meant to encompass such compounds that include multiple ester groups as well as multiple alcohol (hydroxyl) groups in the molecule, and which can include other groups, such as, for example, ether groups, amino groups, sulphydryl groups and the like.

Examples of such suitable polyester polyols include, for example, polyester polyols formed from the reaction of a polycarboxylic acid, such as, a dicarboxylic acid or a tricarboxylic acid (including acid anhydrides) with a polyol, such as, a diol or a triol. The number of ester and alcohol groups, and the relative amount and type of a polyacid and a polyol, are selected such that the resulting polyester polyol compound retains a number of free hydroxyl groups, which can be used for subsequent crosslinking or derivatization in forming the overcoat film-forming material or binder material. For example, suitable polycarboxylic acids include, but are not limited to, adipic acid, pimelic acid, suberic acid, azelaic acid, sebasic acid and the like. Suitable polyols include, but are not limited to, difunctional materials, such as glycols or trifunctional alcohols, such as, triols and the like, including propylenediols, butanediols, hexanediols, glycerines, 1,2,6-hexane triols and the like. Reference is made to U.S. Pub. No. 2009/0130575.

In forming the film-forming material or binder for the overcoating layer in embodiments where the film-forming material or binder is a polyester polyol, a polyol, or a combination thereof, any suitable crosslinking agent, a catalyst and the like can be included in known amounts for known purposes. For example, a crosslinking agent or an accelerator, such as, a trioxane, a melamine crosslinking agent, mixtures thereof and so on, can be included with a polyester polyol reagent to form an overcoating layer. Incorporation of a crosslinking agent or accelerator provides reaction sites to interact with the polyester polyol to provide a branched, crosslinked structure. Where melamine compounds are used, they can be suitably functionalized to be, for example, melamine formaldehyde, methoxymethylated melamine compounds, such as glycouril formaldehyde, benzoguanamine formaldehyde and the like.

Crosslinking can be accomplished by heating in the presence of a catalyst. Thus, the solution of the polyester polyol can also include a suitable catalyst. Typical catalysts include, for example, oxalic acid, maleic acid, carbollylic acid, ascor-

## 11

bic acid, malonic acid, succinic acid, tartaric acid, citric acid, p-toluenesulfonic acid, methanesulfonic acid and the like and mixtures thereof.

If desired or necessary, a blocking agent also can be included. A blocking agent can be used to "tie up" or block an acid effect to provide solution stability until an acidic catalyst function is desired. Thus, for example, the blocking agent can block an acid effect until the solution temperature is raised above a threshold temperature. For example, some blocking agents can be used to block an acid effect until the solution temperature is raised above about 100° C. At that time, the blocking agent dissociates from the acid and vaporizes. The unassociated acid is then free to catalyze polymerization. Examples of such suitable blocking agents include, but are not limited to, pyridine and commercial acid solutions containing such blocking agents.

Any suitable alcohol solvent may be employed for the film-forming material. Typical alcohol solvents include, for example, butanol, propanol, methanol, 1-methoxy-2-propanol and the like and mixtures thereof. Other suitable solvents that can be used in forming the overcoating layer solution include, for example, tetrahydrofuran, monochlorobenzene and mixtures thereof. The solvents can be used in addition to, or in place of, the above alcohol solvents.

A suitable hole transport material may be utilized in the overcoat layer to improve charge transport mobility of the layer. The hole transport material can be, for example, a biphenyl or terphenyl hole transporting molecule, such as, a biphenyl or terphenyl diamine hole transporting molecule. In some embodiments, the hole transporting molecule is soluble in alcohol to assist in application along with the polymer or film-forming material or binder in solution form. However, alcohol solubility is not required and the combined hole transporting molecule and film-forming material or binder can be applied by methods other than in solution, as needed.

An overcoat may comprise a dispersion of nanoparticles, such as silica, metal oxides, waxy polyethylene particles, polytetrafluoroethylene (PTFE) and the like. The nanoparticles may be used to enhance lubricity, scratch resistance and wear resistance of an overcoat layer. In some embodiments, the nanoparticles are comprised of nanopolymeric gel particles of crosslinked polystyrene-n-butyl acrylate dispersed or embedded in a film-forming material, binder or polymer matrix.

In some embodiments, an overcoat layer may comprise a charge transport molecule or component. The charge transport molecule may be present in some embodiments in an amount from about 1% to about 60% by weight of the total weight of an overcoat layer.

A copolymer of first propylene monomer and a second hydrophilic monomer is included in an overcoat of interest.

The propylene monomer can be substituted as taught herein, generally with substituents that retain the hydrophobic nature of the monomer. Hence, a suitable substituent is a hydrocarbon, whether linear, cyclic or branched.

A suitable hydrophilic monomer that can be used is one carrying, for example, a hydroxyl group, a carboxyl group, a carbonyl group, an aldehyde group, an ester group, an amino group, a sulfoxide group, a thiol group and so on, combinations thereof and any other substituent with hydrophilic properties. A hydrophilic monomer of interest is one which can comprise a hydrocarbon, which may be modified or substituted, for example, to contain a heteroatom, such as, S, O, N or P, for example, wherein the hydrocarbon can be aliphatic, cyclic, aromatic, branched or combinations thereof, and may contain from 1 to about 20 carbons atoms. Examples of suit-

## 12

able monomers include a glycol, such as, ethylene glycol, propylene glycol, butylene glycol and so on; an ether, such as, ethylene oxide, tetrahydrofuran and so on; an aldehyde, such as, formaldehyde and so on; an ester, such as, a methacrylate, such as, hydroxymethylacrylate, hydroxyethylacrylate, methacrylic acid and so on; an amine, for example, an amide, such as, an acrylamide, such as, dimethyl acrylic acid, sulfo-propyl acrylate, tetrahydrofurfuryl acrylate and so on; and the like.

10 The ratio of the two monomers in the block copolymer can range from about 1% to about 99% (based on moles or weight) for each monomer. The amount of copolymer in the overcoat-forming mixture and in the final overcoat, by weight or volume as appropriate, can range from about 0.5% to about 15 20% about 3% to about 15%; about 4% to about 10%; and so on.

The overcoat solution can contain particles, which can comprise one or more of the reagents or can be created by milling or processing the overcoat-forming mixture. Any 20 such particles can be from about 50 nm to about 1,000 nm in size, from about 100 nm to about 500 nm, or about 300 nm in size. The hydrophilic component of the copolymer may contribute to the particle size stability of the solution in many of the commonly used solvent for such solutions and emulsions, 25 with minimal deterioration or aggregation observed over a period of 1 week to about 26 weeks or more.

In the dried overcoating layer, the composition can include from about 32% to about 88% by weight of film-forming material or binder, from about 2% to about 20% of the copolymer of interest; and from about 64% to about 10% percent by weight of other ingredients. As indicated about, the amount of copolymer can be from about 3% to about 15%; about 4% to about 10%; and so on, with a commensurate adjustment in amounts of the remaining reactants.

35 The thickness of the overcoat layer can depend on the abrasiveness of the charging (e.g., bias charging roll), cleaning (e.g., blade or web), development (e.g., brush), transfer (e.g., bias transfer roll) etc. functions in the imaging device employed and can range from about 1  $\mu$ m or about 2  $\mu$ m to 40 about 10  $\mu$ m or about 15  $\mu$ m or more. A thickness of between about 1  $\mu$ m and about 5  $\mu$ m can be used. Typical application techniques include spraying, dip coating, roll coating, extrusion coating, draw bar coating, wire wound rod coating and the like. The overcoat can be formed as a single layer or as 45 multiple layers. Drying of the deposited coating may be obtained by any suitable conventional technique such as oven drying, infrared radiation drying, air drying and the like.

The dried overcoating can transport holes during imaging. An overcoat may not have a high free carrier concentration as 50 free carrier concentration can increase dark decay. The dark decay of an overcoat can be about the same as that of the unovercoated device.

The basic film-forming materials and other non-photoactive components for constructing a layer, as well as the methods for making, applying and setting the layer on a photoreceptor under construction as described herein can be used for making the other layers taught herein.

## The Anti-Curl Back Coating Layer

An anti-curl back coating may be applied to the surface of 60 a substrate opposite to that bearing the photoconductive layer (s) to provide flatness and/or abrasion resistance, such as, when a web configuration imaging device component is contemplated. An anti-curl back coating layer is known and can comprise a film-forming material or binder, such as, thermoplastic organic polymers or inorganic polymers, that are electrically insulating or slightly semiconductive. The thickness of anti-curl back coating layers generally is sufficient to bal-

ance substantially the total forces of the layer or layers on the opposite side of the substrate. An example of an anti-curl back coating layer is described in U.S. Pat. No. 4,654,284, the disclosure of which is incorporated herein by reference in entirety. A thickness of from about 70  $\mu\text{m}$  to about 160  $\mu\text{m}$  can be used for a flexible device imaging component, although the thickness can be outside that range as a design choice.

Because conventional anti-curl back coating formulations can suffer from electrostatic charge build up due to contact friction between the anti-curl layer and, for example, backer bars, which can increase friction and wear, incorporation of compounds to dissipate charge, such as, nanopolymeric gel particles, into the anti-curl back coating layer can substantially eliminate charge build up. In addition to reducing electrostatic charge build up and reducing wear in the layer, a charge dissipating material, such as, nanopolymeric gel particles, may be used to enhance lubricity, scratch resistance and wear resistance of the anti-curl back coating layer. In some embodiments, the nanopolymeric gel particles are comprised of crosslinked polystyrene-n-butyl acrylate, which are dispersed or embedded in a film-forming material or binder, such as, a polymer or a matrix.

In some embodiments, the anti-curl back coating layer may comprise a charge transport molecule or component. The charge transport molecule may be present from about 1% to about 60% by weight of the total weight of the anti-curl back coating layer.

#### The Undercoat

An undercoat may be present, and can be composed of a binder or a film-forming material or substance, such as, a resin, a casein, a phenolic resin, a polyol, such as an acrylic polyol, an aminoplast resin, a polyvinyl alcohol, a nitrocellulose, an ethylene-acrylic acid copolymer, a polyamide, a polyurethane or a gelatin can be used, and the layer formed, for example, by dip coating. Examples of polyol resins include, but are not limited to, a polyglycol, a polyglycerol and mixtures thereof. The aminoplast resin can be, but is not limited to, urea, melamine and mixtures thereof.

In various embodiments, phenolic resins can be considered condensation products of an aldehyde and a phenol in the presence of an acidic or basic catalyst.

The phenol may be, for example, phenol, alkyl-substituted phenols, such as, cresols and xylenols, halogen-substituted phenols, such as, chlorophenol, polyhydric phenols, such as, resorcinol or pyrocatechol, polycyclic phenols, such as, naphthol and bisphenol A, aryl-substituted phenols, cyclo-alkyl-substituted phenols, aryloxy-substituted phenols and combinations thereof. The phenol may be for example, 2,6-xylenol, o-cresol, p-cresol, 3,5-xylenol, 3,4-xylenol, 2,3,4-trimethyl phenol, 3-ethyl phenol, 3,5-diethyl phenol, p-butyl phenol, 3,5-dibutyl phenol, p-amyl phenol, p-cyclohexyl phenol, p-octyl phenol, 3,5-dicyclohexyl phenol, p-phenyl phenol, p-crotyl phenol, 3,5-dimethoxy phenol, 3,4,5-trimethoxy phenol, p-ethoxy phenol, p-butoxy phenol, 3-methyl-4-methoxy phenol, p-phenoxy phenol, multiple ring phenols and combinations thereof.

The aldehyde may be, for example, formaldehyde, paraformaldehyde, acetaldehyde, butyraldehyde, paraldehyde, glyoxal, furfuraldehyde, propionaldehyde, benzaldehyde and combinations thereof.

The phenolic resin may be, for example, selected from dicyclopentadiene-type phenolic resins, phenol novolak resins, cresol novolak resins, phenol aralkyl resins and combinations thereof, see U.S. Pat. Nos. 6,255,027, 6,155,468, 6,177,219 and 6,156,468, each incorporated herein by reference in entirety. Examples of phenolic resins include, but are not limited to, formaldehyde polymers with p-tert-butylphe-

nol, phenol and cresol; formaldehyde polymers with ammonia, cresol and phenol; formaldehyde polymers with 4,4'-(1-methylethylidene)bisphenol; formaldehyde polymers with cresol and phenol; or formaldehyde polymers with p-tert-butylphenol and phenol. Phenolic resins are commercially available and can be used as purchased or can be modified to enhance certain properties. For example, the phenolic resins can be modified with suitable plasticizers, including, but not limited to, a polyvinyl butyral, a polyvinyl formal, an alkyd, an epoxy resin, a phenoxy resin (bisphenol A or epichlorohydrin polymer), a polyamide, an oil and the like.

Various types of fine particles and metallic oxides can be added to adjust the resistance of the undercoat layer. Examples of such metallic oxides include alumina, zinc oxide, aluminum oxide, silicon oxide, zirconium oxide, molybdenum oxide, titanium oxide, tin oxide, antimony oxide, indium oxide and bismuth oxide. Examples also include fine particles of tin-doped indium oxide, antimony-doped tin oxide and antimony-doped zirconium oxide. A single species of a metallic oxide can be used or two or more types can be used in combination. When two or more are used, the plural oxides can be used in the form of a solution or a fused substance. The average particle size of a metallic oxide can be about 0.3  $\mu\text{m}$  or less, or about 0.1  $\mu\text{m}$  or less. In some embodiments, metallic oxide particles can be surface treated. Surface treatments include, but are not limited to, exposure of the particles to aluminum laurate, alumina, zirconia, silica, silane, methicone, dimethicone, sodium metaphosphate and the like and mixtures thereof.

The solvent used for preparing the undercoat, depending on the presence of additives therein, is one capable of, for example, effective dispersion of inorganic particles and dissolution of the film-forming material or substance. A suitable solvent can be an alcohol, such as those containing 1, 2, 3, 4, 5 or 6 carbons, such as, ethanol, n-propyl alcohol, isopropyl alcohol, n-butanol, t-butanol and sec-butanol. Further, to improve storage ability and particle dispersion, it is possible to use an auxiliary solvent. Examples of such an auxiliary solvent are methanol, benzyl alcohol, toluene, methylene chloride, cyclohexane and tetrahydrofuran.

When particles are dispersed in a binder, resin or film-forming material or substance to prepare an undercoat, the particles can be present in an amount of about 20 wt % to about 80 wt %; from about 30 wt % to about 70 wt %; from about 40 wt % to about 60 wt %; or from about 50 wt % to about 60 wt % of the total weight of undercoat materials.

An ultrasonic homogenizer, ball mill, sand grinder or homomixer can be used to disperse the inorganic particles.

The method of drying the undercoat can be selected as appropriate in conformity with the type of solvent and film thickness. For example, drying by heat can be used.

The film thickness of the undercoat layer can be about 0.1  $\mu\text{m}$  to about 30  $\mu\text{m}$ , or from about 1  $\mu\text{m}$  to about 20  $\mu\text{m}$ , or from about 4  $\mu\text{m}$  to about 15  $\mu\text{m}$ .

Thus, an overcoat of interest is one which does not impact negatively any of the functions normally ascribed to an overcoat and does not impact negatively the overall function of a photoreceptor, however, provides enhanced wear resistance and less torque, thereby extending the life of a photoreceptor. Thus, the electrical properties of a photoconductor or photoreceptor of interest, as evidenced, for example, by PIDC's, are comparable to that of a control photoreceptor not containing an overcoat or lacking a copolymer of interest in an overcoat; and print quality, when in an imaging device, is comparable to that of a control imaging device comprising a photoreceptor lacking an overcoat or an overcoat lacking a copolymer of interest, as evidenced, for example, by ghosting

## 15

studies. When compared to a control, a photoreceptor of interest presents with a wear rate at least about 40% less than control, at least about 50% less than control, at least about 60% less than control, or at least about 70% less than control or more, where a control is a photoreceptor lacking a copolymer of interest in the overcoat, where the wear rate is determined practicing materials and methods known in the art. For example, a test device comprising a bias charge roll (BCR) associated with a photoreceptor can be used. The BCR can be variably charged. The thickness of the coating on a photoreceptor can be determined with a device dedicated to assessing coating thickness, such as those available from Helmut Fischer GmbH, such as, the FISCHERSCOPE™ device. The photoreceptor then is tested in the device for a predetermined number of cycles and the coating thickness is measured and compared to the thickness prior to testing. The wear rate can be determined by dividing the difference in coating thickness by the number of cycles.

An overcoat of interest is used in a photoreceptor as provided herein. Thus, various photoactive and electrically active layers, and other functional layers, along with the overcoat are applied to a substrate to yield a functional photoreceptor as taught herein or as known in the art. An overcoat of interest can be used with any organic photoreceptor independent of the specific substrate, CGL and of the specific other layers that comprise a photoreceptor. The completed photoreceptor comprising an overcoat comprising a copolymer of interest is engaged in an imaging device as known in the art to enable the production of an image product, for example, photocopies. Hence, such an imaging device can comprise a device for producing and removing an imagewise charge on the photoreceptor. The imaging device can contain a developing component for applying a developing composition, such as a finely divided pigmented material to said charge retentive surface of said photoreceptor to yield the image on the surface of said photoreceptor. Such an imaging device also may include an optional transferring component for transferring the developed image from the photoreceptor to another member or a copy substrate or receiving member. The imaging device comprises a device to enable transfer of the image from the photoreceptor to a receiving member, such as, a paper. The imaging device also contains a component for affixing the finely divided pigmented material onto the receiving member. The imaging device also comprises a device to recharge the photoreceptor to remove all charge from the surface thereof to provide a cleared surface on the photoreceptor to accept a new image without any remnants of the prior image.

Various aspects of the embodiments of interest now will be exemplified in the following non-limiting examples.

## EXAMPLES

## Example 1

On a 30 mm thick aluminum drum substrate was deposited an undercoat layer comprising zirconium acetylacetone tributoxide (35.5 parts),  $\gamma$ -aminopropyl triethoxysilane (4.8 parts) and poly(vinylbutyral) BM-S (2.5 parts), which were dissolved in n-butanol (52.2 parts). The resulting solution then was coated by a dip coater onto the aluminum drum substrate and the coating solution layer was preheated at 59° C. for 13 minutes, humidified at 58° C. (dew point=54° C.) for 17 minutes and then dried at 135° C. for 8 minutes. The thickness of the resulting undercoat layer was approximately 1.3  $\mu$ m.

## 16

A photogenerating layer, 0.2  $\mu$ m in thickness comprising chlorogallium phthalocyanine (Type C) was deposited on the above undercoat layer. The photogenerating layer coating dispersion comprised 2.7 g of chlorogallium phthalocyanine Type C pigment, 2.3 g of carboxyl-modified vinyl copolymer, VMCH, available from Dow Chemical Co., 15 g of n-butyl acetate and 30 g of xylene. The resulting mixture was mixed in an Attritor mill with about 200 g of 1 mm Hi-Bea borosilicate glass beads for about 3 hours. The dispersion mixture then was filtered through a 20  $\mu$ m Nylon cloth filter and the solids content of the dispersion was diluted to about 6 weight %.

Subsequently, a 34  $\mu$ m charge transport layer was coated on top of the above photogenerating layer from a solution prepared by dissolving N,N'-diphenyl-N,N'-bis(3-methylphenyl)-1,1'-biphenyl-4,4'-diamine (mTBD, 4 g) and a film-forming polymer binder, PCZ-400 [poly(4,4'-dihydroxy-diphenyl-1-1-cyclohexane carbonate),  $M_w$ =40,000] available from Mitsubishi Gas Chemical Company, Ltd. (6 g), in a solvent mixture of 21 g of tetrahydrofuran (THF) and 9 g of toluene. The CTL was dried in an oven at about 120° C. for about 40 minutes. The resulting CTL layer had a PCZ-400/mTBD ratio of 60/40.

An overcoat composition is formed containing 2.5 grams Joncryl 587 (acrylated polyol from Johnson Polymers Inc.), 3.5 grams Cymel 303, 27 grams 1-methoxy-2-propanol (Dowanol PM) and 3.0 grams N,N'-diphenyl-N,N'-di-[3-hydroxyphenyl]-terphenyl-diamine in a 1 ounce bottle. The components are mixed and the temperature is raised to about 40° C. until a complete solution is achieved. Next, 0.9 grams of p-toluenesulfonic acid/pyridine (8% acid/pyridine complex in 1-methoxy-2-propanol) (0.072 grams acid, 0.75% by weight) as catalyst were added.

The drum was exposed to the overcoating composition using a Tsukiage dip coating apparatus and dried at 155° C. for 40 minutes. The result is an imaging member having an overcoating layer thickness of about 4.5  $\mu$ m.

In other embodiments, an overcoat coating solution was formed by adding to a 240 ml bottle, 80 g 1-methoxy-2-propanol, 10 g of POLYCHEM® 7558-B-60 (an acrylated polyol obtained from OPC Polymers), 4 g of PPG 2K (a polypropylene glycol with a weight average molecular weight of 2,000 as obtained from Sigma-Aldrich), 6 g of CYMEL® 1130 (a methylated, butylated melamine-formaldehyde crosslinking agent obtained from Cytec Industries Inc.), 8 g of N,N'-diphenyl-N,N'-di[3-hydroxyphenyl]-biphenyl-diamine (DHTPD), 5.5 g of an 8% p-toluenesulfonic acid/2-propanol solution and 1.5 g of SICLEAN 3700 (a hydroxylated siliconized polyacrylate available from BYK-Chemie USA). The contents were stirred until a complete solution was obtained.

The photoconductor was overcoated with the above overcoat solution. The resultant overcoated film was dried in a forced air oven for 40 minutes at 155° C. to yield a 4.5  $\mu$ m overcoat, which was substantially crosslinked and insoluble, or substantially insoluble in methanol or ethanol.

Experimental overcoats were prepared as above except that the formulations included 5 weight % of X-10044, a polypropylene-polyethylene glycol block copolymer (Baker Petrolite, average molecular weight of 1300, melting point of 107° C., viscosity at 149° C. of 25 cP and containing 20% ethylene oxide). The mixture was ball milled for 2 hours to yield an emulsion with 200-300 nm sized particulates.

The overcoats were applied to photoconductors as described above.

## Electrical Property Testing

The above prepared photoconductor was compared to an identically prepared photoconductor except that the overcoat of the control lacked a copolymer of interest. The experimental and control devices were tested in a scanner set to obtain photoinduced discharge cycles, sequenced at one charge-erase cycle followed by one charge-expose-erase cycle, wherein the light intensity was incrementally increased with cycling to produce a series of photoinduced discharge characteristic curves (PIDC) from which the photosensitivity and surface potentials at various exposure intensities were measured. Additional electrical characteristics were obtained by a series of charge-erase cycles with incrementing surface potential to generate several voltage versus charge density curves. The scanner was equipped with a scorotron set to a constant voltage charging at various surface potentials. The photoconductors were tested at surface potentials of 700 volts with the exposure light intensity incrementally increased by regulating a series of neutral density filters; the exposure light source was a 780 nm light emitting diode. The xerographic simulation was conducted in an environmentally controlled light tight chamber at dry conditions (10% relative humidity and 22° C.).

The experimental photoconductors had a residual potential of about 150 V as compared to about 170 V for control photoconductors that did not contain a copolymer of interest in the overcoat. Hence, incorporating a copolymer of interest in the overcoat did not adversely impact the electrical properties of the photoconductor and reduced surface potential.

## Wear Test

Wear tests of the photoconductors of Comparative Examples 1 and 2 and Example 1 were performed using an in house wear test fixture (biased charging roll (BCR) with charging of peak to peak voltage of 1.45 kilovolts. The total thickness of each photoconductor was measured via Permascope (Helmut Fischer) before each wear test was initiated. Then the photoconductors were separately placed in the wear fixture for and tested 50 kilocycles. The total photoconductor thickness was measured again with the Permascope, and the difference in thickness was used to calculate wear rate (nanometers/kilocycle) of the photoconductors. The smaller the wear rate, the more wear resistant was the photoconductor. The wear rate data is summarized in Table 1.

TABLE 1

|                              | Wear Rate<br>(Nanometers/Kilocycle) |
|------------------------------|-------------------------------------|
| Control, no copolymer        | 15                                  |
| Experimental, with copolymer | 12                                  |

When a copolymer of interest was incorporated into the overcoat, the wear rate was reduced as compared to control. Torque Test

Drums were cycled for 30 minutes under conditions of hyper mode test of charge and erase cycling with a bias charge roller charging device. The ozone evacuation hoses were disconnected to produce maximal corona induction. After cycling, the drum was placed in the black print station of a Copeland 3545 printer. A standard print test was requested. If printing did not occur or fault codes were observed, the drum was considered a failure.

Control drums carrying control overcoats failed the test. Drums with no overcoat passed the test. Experimental drums with an overcoat containing a copolymer of interest passed the test.

## 5 Ghosting Measurement

Photoconductors were acclimated at room temperature for 24 hours before testing in a closed container chamber (85° F. and 80% humidity) for A ghosting. Print testing was accomplished in the Xerox Corp. WorkCentre™ Pro C3545 using the K (black toner) station at t of 500 print counts (t=500 is the 500<sup>th</sup> print) and in the CMY station of the color WorkCentre™ Pro C3545 which operated from t of 0 to t of 500 print counts. The prints for determining ghosting characteristics include placing an X symbol or letter on a half tone image.

10 When X is invisible, the ghost level is assigned Grade 0; when X is barely visible, the ghost level is assigned Grade 1; and Grade 2 to Grade 5 refer to the level of visibility of X with Grade 5 being a dark and visible X. Ghosting levels were visually measured against an empirical scale, the lower the ghosting grade (absolute value), the better the print quality.

15 Photoconductors were also acclimated in J zone conditions (75° F. and 10% humidity) in a closed container chamber for 24 hours before print tested, as above, to assess J zone ghosting.

20 Very low ghosting was observed in the A and J zones for both control and experimental photoconductors.

## Long Term Cycling

25 The photoconductors were also tested for wear resistance under long term cycling conditions. The photoconductors were assessed under both J and A zone conditions.

30 Under both conditions, stable cycling was observed up through 200,000 cycles, with surface potential remaining fairly static after about 50,000 cycles.

35 All references cited herein are herein incorporated by reference in entirety.

40 It will be appreciated that variants of the above-disclosed and other features and functions, or alternatives thereof, may be combined with other and different systems or applications. Various presently unforeseen or unanticipated alternatives, changes, modifications, variations or improvements subsequently may be made by those skilled in the art to and based on the teachings herein without departing from the spirit and scope of the embodiments, and which are intended to be encompassed by the following claims.

45 The invention claimed is:

1. A photoreceptor overcoat comprising a film-forming material, a charge transport material and a copolymer, wherein monomers thereof are a first propylene monomer and a second hydrophilic monomer, wherein the hydrophilic monomer comprises ethylene glycol.

50 2. The overcoat of claim 1, wherein said ethylene glycol comprises about 20% of said copolymer.

3. The overcoat of claim 1, wherein said copolymer is a block copolymer.

55 4. A photoreceptor comprising the overcoat of claim 1.

5. The overcoat of claim 4, wherein said ethylene glycol comprises about 20% of said copolymer.

60 6. The photoreceptor of claim 4, wherein said copolymer is a block copolymer.

7. An imaging device component comprising the photoreceptor of claim 4.

8. An imaging device comprising the component of claim 7.

65 9. An imaging device comprising a photoreceptor comprising an overcoat comprising a film-forming material, a charge transport material and a copolymer comprising a first propylene monomer and a second hydrophilic monomer, wherein

**19**

said photoreceptor has a wear rate about 20% less than of a photoreceptor lacking an overcoating comprising a first propylene monomer and a second hydrophilic monomer, wherein the hydrophilic monomer comprises ethylene glycol.

**10.** A method of reducing the wear rate of a photoreceptor comprising adding a copolymer comprising a first propylene monomer and ethylene glycol to an overcoat of said photoreceptor, said overcoat comprising a film-forming material and a charge transport material. 5

\* \* \* \* \*

10

**20**